# EUROPEAN PATENT SPECIFICATION

(11) **EP 1 359 246 B1**
(45) Date of publication and mention of the grant of the patent: **05.11.2008**
(21) Application number: 03005096.7
(22) Date of filing: 07.03.2003
(51) Int. Cl.: D06M 13/127, D06M 13/21, D06M 13/342, D06P 1/00, D06P 1/651, D06P 3/14

(54) **Method for controlling coloring of fiber**
Verfahren zur Regulierung der Faserfärbung
Procédé de régulation de la coloration d' une fibre

(30) Priority: 02.05.2002 JP 2002130613
(43) Date of publication of application: 05.11.2003
(73) Proprietor: Kurabo Industries Ltd., Japan, Kurashiki-shi, Okayama 710-0054 (JP); Fukuoka Prefectural Government, Japan, Hakata-ku, Fukuoka 812-8577 (JP); Pyramid Corporation, Japan, Kurume-shi, Fukuoka 830-0063 (JP)
(72) Inventor: Donowaki, Kiyoshi, Chikushino-shi, Fukuoka 818-0004 (JP); Nakamura, Masashi, Kurume-shi, Fukuoka 839-0808 (JP); Ohshima, Kunihiro, Neyagawa-shi, Osaka 572-0823 (JP); Miyagai, Kiyotaka, Neyagawa-shi, Osaka 572-0823 (JP); Kogoh, Kazuhiko, Neyagawa-shi, Osaka 572-0823 (JP); Aoyama, Yasuhiro c/o Kurabo Industries Ltd., Tokyo 103-0023 (JP)
(74) Representative: Jönsson, Hans-Peter

(56) References cited:
- DE-A- 19 717 224
- DE-A- 19 820 894
- PATENT ABSTRACTS OF JAPAN vol. 2000, no. 19, 5 June 2001 (2001-06-05) & JP 2001 055672 A (FUKUOKA PREFECTURE), 27 February 2001 (2001-02-27)

## Description

### 1. Field of the Invention

The present invention belongs to the technical field for coloring fibers and relates to the technique for controlling the developed color, particularly in the technique for coloring animal fibers etc. without using dyes.

### 2. Description of the prior art

Some novel methods for coloring fibers using fiber itself as the chromophoric material by converting tryptophan being contained in animal fiber etc. to chromophore components are known, differing from the method for dyeing animal fiber using the synthetic dyes in the past. Japanese Patent Application Laid-Open No.2001-55672 discloses that various colors can be brought out from acid-treating animal fiber together with aldehyde compounds, that the obtained color has durability against sweat, abrasion and washing, and that the color depends on the combination of the acid and the aldehyde.

In above prior art, however, the controlling technology for making deep color is not satisfactory, and there is still the problem for the industrialization because the reaction must be conducted in an organic solvent system.

DE 198 20 894 A1 describes a 2-component agent for colorizing fibres consisting of (a) a first component containing thiobarbituric acid and/or its derivatives and (b) a second component containing a carbonyl compound being selected from the group of saturated dialdehydes, saturated diketones, saturated ketoaldehydes, unsaturated dialdehydes, unsaturated diketones, unsaturated ketoaldehydes, monoaldehydes with one or more chromophoric groups, monoketones with one or more chromophoric groups and quinones. Also described is a process for colorizing fibres using this 2-component agent.

DE 197 17 224 A1 discloses the use of aliphatic unsaturated dialdehydes for colorizing keratin containing fibres, especially human hair.

### SUMMARY OF THE INVENTION

The present invention is to provide a controlling technology which makes deeper-coloring possible and a method in which coloring and deeper-coloring are conducted in a water system.

The present invention provides to a method for controlling color development of fiber in a coloring method of fiber in which a tryptophan-containing fiber is colored with an aldehyde compound, comprising;
a first step: a process for treating a fiber which contains tryptophan constitutionally or in which tryptophan is introduced from outside with an acid and an aldehyde compound selected from benzaldehyde or its derivatives; and a second step : a process for treating the fiber treated in the first step with an oxidizer in the presence of an acid.

### DETAILED DESCRIPTION OF THE PREFERRED EMBODIMENTS

The present invention relates to a method for controlling color development of fiber in a coloring method of fiber in which a tryptophan-containing fiber is colored with aldehyde compound, comprising;
a first step: a process for treating a fiber which contains tryptophan constitutionally or in which tryptophan is introduced from outside with an acid and an aldehyde compound selected from benzaldehyde or its derivatives; and
a second step : a process for treating the fiber treated in the first step with an oxidizer in the presence of an acid.

Particularly, the present invention relates to the above method for controlling color development of fiber, wherein the benzaldehyde derivatives are water-soluble benzaldehyde derivatives.

In the present invention, "controlling color development of fiber" or "controlling coloring of fiber" means to control coloring conditions such as a kind of color and concentration of color.

According to the method for controlling the coloring of fiber in the present invention, tryptophan-containing fibers are treated with an acid and an aldehyde compound selected from benzaldehyde or its derivatives in the first step. In the treatment of this step, the fiber is made contact with a treating solution containing an acid and an aldehyde compound so that the tryptophan in the fiber and aldehyde compound may react to be condensed and that the aldehyde compound combines to the fiber. In this treating solution, a concentration of acid is preferably adjusted to 10⁻⁵ to 2N, more preferably 10⁻² to 1N.

While the addition reaction between tryptophan and aldehyde compound selected from benzaldehyde or its derivatives is promoted by adjusting the acid concentration in the treating solution within the above-mentioned range, it is considered that the color is developed by the formation of conjugated double bond between tryptophan and aldehyde compound as the result of the oxidation of aldehyde compound added to tryptophan. Especially, in the case that the aldehyde compound is an aromatic compound, when the aromatic aldehyde compound added to tryptophan is oxidized, an aromatic ring in aromatic aldehyde is converted to a quinoid structure, so that a conjugated double bond is formed between tryptophan and aldehyde, resulting in coloring development.

The coloring can be controlled to yellow colors having characteristic absorption wave-length at 400 - 500nm in the case that the aromatic ring can be converted to an o-quinoid structure, and to the colors from red to blue or green having absorption at 500 - 800nm in the case that it can be converted to a p-quinoid structure. However the present invention is not restricted to the above. The control can be made by changing kind, number, position etc. of the functional group in benzaldehyde derivatives.

However, in this first step, the oxidation is restricted. Only the first step can not achieve satisfactory color development with sufficient concentration. In this step, the oxidation reaction is promoted when the temperature is raised, but the fiber is decomposed or dissolves by the acid. Therefore, it is preferable that the treatment should be conducted without heating. The temperature range is preferably 20 - 90°C, more preferably 20 - 70°C.

The treating solution is obtained as an aqueous solution by using water-soluble compounds as benzaldehyde derivatives. In this case, the aggravation of the working environment according to solvents can be prevented and the possibility of fire or explosion also disappears, and so the industrial process is possible, being very favorable.

As described above, though some degree of coloring is achieved in the first step, the color concentration is in general insufficient merely in the first step and the deepening process of the color is required to make the color deeper. For deepening of the color, the fiber treated in the first step is treated with oxidant in the presence of an acid in the second step. Through this step, the aldehyde compound bound to tryptophan is more perfectly oxidized and the concentration of aldehyde which can form the conjugated double bond with tryptophan increases. As the result, the developed color becomes deeper and deeper coloring is attained. When the aldehyde compound is an aromatic aldehyde, a quinoid structure is formed as mentioned above and this concentration increases with the treatment by an oxidant.

The coloring can be controlled to yellow colors having characteristic absorption wave-length at 400 - 500nm in the case that the aromatic ring can be converted to an o-quinoid structure, and to the colors from red to blue or green having absorption at 500 - 800nm in the case that it can be converted to a p-quinoid structure. However the present invention is not restricted to the above. The control can be made by changing kind, number, position etc. of the functional group in the benzaldehyde derivatives.

The transfer from the first step to the second step may be conducted by the way that the fiber colored in the first step is once washed and dried and then subjected to the second step, or washed and then subjected to the second step without drying.

The treatment in the second step may be conducted at 20 - 90°C, preferably at 20 - 70°C in the same way as in the first step.

When above-mentioned treating temperature is used, the treating time is usually 1-6 hrs in the first step, and 1-24 hrs in the second step.

The fiber contacted with a treating solution in the second step may be kept immersed in the treating solution until the reaction finishes, or may be taken out of the treating solution and be subjected to reaction in the state that the fiber sufficiently contains the treating solution by immersion.

After finishing the treatment in the second step, the fiber may be sufficiently washed with an adequate cleaning solution which can get rid of aldehyde compounds, such as water or water/methanol mixture, and then may be air-dried at ordinary temperature or may be dried at such a temperature as quality of the fiber would not be spoiled.

The principle of the present invention is applied for coloring fibers containing tryptophan constitutionally or extrinsically. It is particularly advantageous to color the fibers having tryptophan constitutionally, that is, protein fibers. Protein fibers to be applied are generally animal fibers, particularly wool or silk. The examples of protein fibers other than animal fibers are protein fibers regenerated from casein, zein, peanut protein etc. as raw materials. The present invention can be applied for coloring these fibers.

The method of the present invention can be also applied for coloring the fibers containing tryptophan extrinsically, that is, such fibers as tryptophan is introduce from outside, in addition to the fibers containing tryptophan constitutionally such as animal fibers (protein fibers). For example, by introducing and binding tryptophan to hydroxide group in cellulose constructing cotton in a coupling reaction, such cotton fiber can be colored according to the present invention.

In the present invention, "fiber" means not only fiber itself, but also fiber products such as cloth, clothing and the like.

Aldehyde compounds used in the present invention are selected in combination with acids according to the required color, and particularly benzaldehyde or its derivatives having benzaldehyde as the basic skeleton are preferable. By using water-soluble aromatic benzaldehyde compounds or benzaldehyde derivatives, the coloring reaction and deeper-coloring reaction can be conducted in water system.

The water-soluble derivatives of benzaldehyde are exemplified by 4-hydroxybenzaldehyde, 4-dimethylaminobenzaldehyde, 2,4,6-trimethoxybenzaldehyde, 3,4-dihydroxybenzaldehyde and a mixture thereof, with no intention to limit them to restricted examples.

An amount of aromatic aldehyde to be used is determined by depth of color required for colored fiber and amount of tryptophan contained in the fiber. The color development occurs by the reaction between tryptophan and aldehyde compound, and it is expected that one mole of aldehyde compound reacts with two moles of tryptophan in maximum. Thus, the reaction between aldehyde compound and tryptophan is theoretically saturated with aldehyde of the half amount by mole of existing tryptophan, but the amount of aldehyde compound to be used should be properly determined by the depth of color required. Generally, as one example, about 0.5 to 5% by weight based on total weight of fibers can be used.

In the present invention, an acid which is used together with aldehyde compounds in the first step, is preferably the one belonging to strong acids, but should not be the one which may dissolve the fiber. The preferable examples of the acids which can bring about the effect of the present invention on the fibers without giving the fibers damage, are the acids obtained by diluting strong acids such as trifluoroacetic acid, dichloroacetic acid, hydrochloric acid, sulfuric acid and oxalic acid with water or weak acid such as acetic acid.

The ratio of acid and aldehyde compound is not particularly restricted, but it is determined by the degree of shade of color desired.

The acid used in the second step may be the same acid as used in the first step. The concentration of acid in the treating bath is 10⁻⁵N to 0.5N in the second step.

In the second step, aromatic aldehydes which still maintains non-oxidized state after the first step are oxidized with the action of oxidizer so that the aromatic ring forms quinoid structure, resulting in that the color development becomes deeper. The oxidizer to be available may be water-nonsoluble oxidizers or water-soluble oxidizers. From the viewpoint of treatment in water system, the water-soluble oxidizers are preferable. The examples of the water-soluble oxidizer are hydrogen peroxide, peracetic acid, monopersulfates etc. Particularly preferable oxidizers are hydrogen peroxide and monopersulfates. A concentration of the oxidizer is 10⁻⁵% to 5% by weight in treating solution.

In the treating solution of the first step, a salting-in agent may be added to make it easy for aldehyde compound to dissolve in water. The salting-in agents are exemplified by halides of alkaline metals or halides of alkaline earth metals, such as calcium chloride, lithium chloride, sodium chloride and lithium bromide. Particularly preferable salting-in agents are calcium chloride, sodium chloride and lithium bromide.

### EXAMPLES

The following examples illustrate the features of the present invention.

### Examples 1-4

### [The first step treatment]

Benzaldehydes derivatives listed in Table 1 were dissolved to give concentration of 2% by weight in 60ml of 1N-hydrochloric acid containing 10% by weight of acetic acid and 20% by weight of calcium chloride, and 6g of untreated wool fabric was dipped in this solution. The solution was raised to 60°C in this condition and subjected to reaction for 3 hrs. After reaction, the wool fabric was washed with water and dried at 80°C to give a colored wool fabric. The degree of coloring was measured using "Spectro Color Meter SE 2000" manufactured by Nippon Denshi Kogyo K.K. and a diagram of L*a*b* was obtained. The results were shown in Table 1.

### [The second step treatment]

The wool fabric treated in the first step was dipped in a mixed solution containing 20ml of 0.5N-sulfuric acid and 1ml of 35%conc.-hydrogenperoxide and was maintained in the solution for 2 hrs at room temperature. The fabric was taken out of the solution and kept in air overnight to give the fiber colored deeper. The colored degree was measured in the same way as described above and the results were shown in Table 1.

The fact that a L* value expressing brightness was lower in the second step than in the first step shows that the deeper coloring was developed in the second step. Table 1

| Ex. | Benzaldehyde derivatives | 1st Step | | | 2nd Step | | |
|---|---|---|---|---|---|---|---|
| | | L* | a* | b* | L* | a* | b* |
| 1 | 4-hydroxy benzaldehyde | 78.470 | 5.7100 | 19.510 | 60.290 | 14.280 | 14.230 |
| 2 | 4-dimethylamino benzaldehyde | 51.630 | 6.4300 | 6.5200 | 37.800 | -1. 9900 | -10.080 |
| 3 | 2,4, 6-trimethoxy benzaldehyde | 66.600 | -0. 6700 | 9.9800 | 52.000 | -0.790 | -6.5700 |
| 4 | 3, 4-dihydroxy benzaldehyde | 70.150 | 10.440 | 28.310 | 48.690 | 16.420 | 14.470 |

According to the present invention, the deeper coloring of fibers, which has been difficult to control, has become easy, and the method for coloring of tryptophan-containing fibers has become easier to be controlled. According to the present method, the deeper coloring has become possible with less damage of fibers. In addition, according to the present method, the treatment in water medium has become possible and therefore the present method is suitable for an industrial process. It is also possible to decrease concentration of acid in the treatment of the first step.

## Claims

1. A method for controlling color development of fiber in a coloring method of fiber in which a tryptophan-containing fiber is colored with aldehyde compound, comprising;
a first step: a process for treating a fiber which contains tryptophan constitutionally or in which tryptophan is introduced from outside with an acid and an aldehyde compound selected from benzaldehyde or its derivatives; and
a second step: a process for treating the fiber treated in the first step with an oxidizer in the presence of an acid.

2. The method for controlling color development of fiber according to claim 1, wherein said benzaldehyde derivatives are water-soluble benzaldehyde derivatives.

3. The method for controlling color development of fiber according to claim 2, wherein said water-soluble benzaldehyde derivatives are selected from a group consisting of 4-hydroxybenzaldehyde, 4-dimethylaminobezaldehyde, 2,4,6-trimethoxybenzaldehyde, 3,4-dihydroxybenzaldehyde and a mixture thereof.

4. The method for controlling color development of fiber according to any one of the preceding claims, wherein the process for treating the fiber in the first step is carried out in an aqueous solution having a content of the acid in the range between 10⁻² and 1 N and a content of the acid in the second step is in the range between 10⁻⁵ and 0.5 N.

## Patentansprüche

1. Verfahren zur Steuerung der Farbentwicklung einer Faser bei einem Faserfärbeverfahren, bei dem eine tryptophanhaltige Faser mit einer Aldehydverbindung gefärbt wird, umfassend:
einen ersten Schritt: ein Verfahren zur Behandlung einer Faser, die Tryptophan als konstitutionellen Bestandteil enthält oder in die Tryptophan von außen eingeführt wurde, mit einer Säure und einer Aldehydverbindung, die aus Benzaldehyd oder seinen Derivaten ausgewählt ist; und
einen zweiten Schritt: ein Verfahren zur Behandlung der im ersten Schritt behandelten Faser mit einem Oxidationsmittel in Gegenwart einer Säure.

2. Verfahren zur Steuerung der Farbentwicklung einer Faser gemäß Anspruch 1, wobei die Benzaldehyd-Derivate wasserlösliche Benzaldehyd-Derivate sind.

3. Verfahren zur Steuerung der Farbentwicklung einer Faser gemäß Anspruch 2, wobei die wasserlöslichen Benzaldehyd-Derivate aus der Gruppe ausgewählt sind, die aus 4-Hydroxybenzaldehyd, 4-Dimethylaminobenzaldehyd, 2,4,6-Trimethoxybenzaldehyd, 3,4-Dihydroxybenzaldehyd und einem Gemisch davon besteht.

4. Verfahren zur Steuerung der Farbentwicklung einer Faser gemäß einem der vorstehenden Ansprüche, wobei das Verfahren zur Behandlung der Faser im ersten Schritt in einer wässrigen Lösung durchgeführt wird, die einen Säuregehalt im Bereich von 10⁻² bis 1 N aufweist, und der Säuregehalt im zweiten Schritt im Bereich von 10⁻⁵ bis 0,5 N liegt.

## Revendications

1. Procédé pour commander le développement de couleur d'une fibre dans un procédé de coloration de fibres dans lequel une fibre contenant du tryptophane est colorée avec un composé aldéhyde, comprenant:
une première étape: un procédé dans lequel une fibre contenant du tryptophane comme composant constituant ou dans laquelle le tryptophane a été introduit de l'extérieur est traitée avec un acide et un composé aldéhyde choisi parmi le benzaldéhyde ou ses dérivés; et
une seconde étape: un procédé dans lequel la fibre traitée dans la première étape est traitée avec un agent oxydant en présence d'un acide.

2. Procédé pour commander le développement de couleur d'une fibre selon la revendication 1, dans lequel lesdits dérivés de benzaldéhyde sont des dérivés de benzaldéhyde solubles dans l'eau.

3. Procédé pour commander le développement de couleur d'une fibre selon la revendication 2, dans lequel lesdits dérivés de benzaldéhyde solubles dans l'eau sont choisis dans le groupe constitué par le 4-hydroxybenzaldéhyde, le 4-diméthylaminobenzaldéhyde, le 2,4,6-triméthoxybenzaldéhyde, le 3,4-dihydroxybenzaldéhyde et un mélange de ceux-ci.

4. Procédé pour commander le développement de couleur d'une fibre selon l'une quelconque des revendications précédentes, dans lequel le procédé de traitement de fibre dans la première étape est réalisé dans une solution aqueuse ayant une teneur en acide comprise dans la gamme allant de 10⁻² à 1 N, et la teneur en acide dans la seconde étape est comprise dans la gamme allant de 10⁻⁵ à 0,5 N.
